

May 23, 1944.

R. S. DEAN

2,349,577

CONTROL MEMBER

Filed Nov. 21, 1941

2 Sheets-Sheet 1



COEFFICIENT OF LINEAR  
EXPANSION 10<sup>-6</sup> cm/cm/deg.C.

INVENTOR.  
*Reginald S. Dean*

BY

*McLaughlin & Wallenstein*

ATTORNEYS

May 23, 1944.

R. S. DEAN

2,349,577

CONTROL MEMBER

Filed Nov. 21, 1941

2 Sheets-Sheet 2



INVENTOR  
Reginald S. Dean

BY

McLaughlin & Wallenstein

ATTORNEYS

## UNITED STATES PATENT OFFICE

2,349,577

## CONTROL MEMBER

Reginald S. Dean, Salt Lake City, Utah, assignor  
to Chicago Development Company, Chicago,  
Ill., a corporation of Illinois

Application November 21, 1941, Serial No. 419,872

21 Claims. (Cl. 297—15)

This invention relates to thermostatic elements in the form of alloys of a high coefficient of expansion. It relates more, in particular, to alloys having a high tensile strength and yield point in combination with a high coefficient of linear expansion and to thermostatic metals, particularly bimetals, of which the high expansion members are the manganese, nickel, copper alloys disclosed hereinafter. The alloys or thermostatic metals to which the invention relates have as constituents manganese, nickel and copper.

The invention will be explained, in part, by reference to the accompanying drawings, wherein

Fig. 1 is a ternary diagram showing a number of curves illustrative of the linear expansion characteristics of the alloys; and

Fig. 2 is a similar diagram identifying certain areas.

In Fig. 1, I have illustrated the coefficients of linear expansion by lines of equal coefficients drawn on a ternary diagram representing the three component system, manganese, nickel and copper. Although the manganese, copper, nickel alloys disclosed herein are highly useful for the purposes of the present invention without any heat treatment, those illustrated in the diagram were prepared by quenching from 900 degrees C. and subsequently cold working them. The coefficients of expansion of the alloys as quenched and cold worked are not greatly affected by subsequent heat treatment. In the following table, I show the coefficients of linear expansion of several specific alloys in both the quenched and cold worked states, and also after aging at 450 degrees C. In this particular case, the measurements were made from room temperature to 100 degrees C.

Coefficient of linear expansion  $\times 10^{-6}$  cm./cm./° C.

| Composition |    |    | Quenched and cold worked | Quenched from 900° | 450° |
|-------------|----|----|--------------------------|--------------------|------|
| Mn          | Ni | Cu |                          |                    |      |
| 75          | 20 | 5  | 24.7                     | 26.3               | 25.3 |
| 75          | 5  | 20 | 23.6                     | 24.5               | 22.5 |
| 25          | 10 | 65 | 16.8                     | 19.1               | 16.4 |
| 20          | 20 | 60 | 14.9                     | 17.5               | 15.2 |
| 70          | 30 | 0  | 22.5                     | 22.6               | 21.9 |
| 80          | 5  | 5  | 14.5                     | 22.1               | 15.6 |
| 72          | 10 | 18 | 26.1                     | 28.3               | 21.5 |

In addition to the high coefficient of linear expansion which is illustrated by the values given, I have found that these alloys possess other val-

uable properties which make them useful in articles where high coefficients of linear expansion are necessary. As indicated by the table, certain of the alloys of my invention may be hardened by heat treatment. The extent of this hardening and the preferred heat treatment for bringing it about differ in different composition ranges.

In Fig. 2, I have illustrated several ranges of composition which have been designated by outlining areas identified by the letters A, B and C. In the composition range within the area A, I have found that a suitable treatment to develop high strength and yield point is to heat to a temperature of about 900 degrees C., quench and then age at about 450 degrees C. A cold working step or steps may be introduced between the quenching and aging steps. As a result of this heat treatment, these alloys may be given tensile strength of 150,000 to 200,000 pounds per square inch and a yield point of 75% of the tensile strength. Even higher tensile strengths may be obtained, but the yield point then as a rule is closer to the value for ultimate tensile strength.

In the composition range B, a suitable heat treatment is to quench the alloys from about 900 degrees C. and then age at a temperature of 700 degrees C. Under these conditions, these alloys have greatly increased hardness imparted to them.

In the composition range C, a suitable heat treatment is to quench the alloys from about 900 degrees C. and age them at a temperature of 600 degrees C. With this treatment of the alloys in this range, tensile strengths of 120,000 pounds per square inch may be obtained. I have found that the alloys of my invention possess high electrical resistance and that the electrical resistance may be considerably enhanced by quenching from a temperature of about 900 degrees C. The quenched alloy may be cold worked without adversely affecting its electrical resistance.

I have found that there is an approximate parallelism between electrical resistance and coefficient of linear expansion in the alloys of my invention. I have found, for example, that alloys having electrical resistances between 170 and  $200 \times 10^{-6}$  ohms/cm.<sup>3</sup> show a coefficient of linear expansion in excess of  $20 \times 30^{-6}$  cm./cm./degree C. and that the alloys having an electrical resistance of less than  $150 \times 10^{-6}$  ohms have a coefficient of linear expansion of approximately  $15 \times 10^{-6}$  cm./cm./degree C.

I have found that aging at 450 degrees C. adversely affects the electrical resistance in the

alloys within the composition range indicated by the area A in Fig. 2, while in the area B of Fig. 2, the electrical resistance may be greatly enhanced by heat treatment. A suitable treatment to develop very high electrical resistances in alloys within the area B, is to quench from 900 degrees C. and reheat at a temperature of 700 degrees C. for several hours. By this treatment, electrical resistances as high as  $2000 \times 10^{-6}$  ohms can be obtained.

I have found that the manganese, nickel, copper alloys have relatively low temperature coefficients of electrical resistance. This property is especially low in the alloys having coefficients of linear expansion of approximately  $15 \times 10^{-6}$  cm./cm./degree C. and in the alloys having coefficients of linear expansion of more than  $20 \times 10^{-6}$  cm./cm./degree C. All of these alloys have a relatively high modulus of elasticity. Many of them have a modulus of more than 20,000,000 pounds per square inch. These alloys also possess high fatigue strength. These various properties, combined with high coefficients of linear expansion, make the alloys of my invention particularly useful, for example, as bi-metal strips for temperature control work. In such strips it is important not only to have a high coefficient of linear expansion, but also to have a high yield point and modulus of elasticity. High vibration damping capacity is also of value in materials for this use, since it may prevent chattering of the electrical contacts which are frequently made by the use of such strips. A high coefficient of electrical resistance combined with a high coefficient of linear expansion is very useful in certain types of electrical equipment where it is advantageous to utilize the expansion of a member when it is heated by the passage of an electrical current. The properties of these alloys make them of extreme value in various types of temperature and electrical control members in the various industries in which such control members are used.

As an illustration, reference may be made to bi-metallic strips responsive to temperature changes. A conventional type of strip is one consisting of a low expansion component in the form of a high nickel alloy such as Invar, with a high expansion component such as brass, copper or certain nickel, chromium, iron alloys. By employing a high nickel alloy, such as Invar (64% iron, 36% nickel), having a low coefficient of linear expansion, and one of the alloys of my invention having a coefficient of linear expansion of about 25 or higher  $\times 10^{-6}$  cm./cm./degree C., I can obtain about twice the movement per unit of temperature change as compared with the conventional strip. I may also use an ordinary steel in combination with the high expansion alloys of my invention, and obtain considerable advantages. The low expansion component or member, while most suitably Invar or other iron-nickel alloys having a high content of nickel, of the order of about 36% or higher, may be any other metal or alloy, illustrative examples thereof being disclosed in Patents Nos. 1,947,065 and 1,991,438. My alloys may be produced with a modulus of elasticity of better than twenty million, a figure substantially in the steel range. In producing the bi-metallic strips, they may be welded, fused, brazed or otherwise handled in accordance with the usual practices. While I have mentioned bi-metallic strips as illustrative, it will be understood that such strips or members may comprise more than two laminae, or the

temperature responsive device may take the form of known mechanical arrangements such as a rod within a tube.

Another type of control unit is one where the expansion of a single material, e. g., a bar, is utilized for control purposes. With the high electrical resistance obtainable with our alloys, the control member may carry a current and may be used in a circuit where rise of temperature produced through resistance of the member causes such linear expansion of the control member as to open a set of contacts and interrupt the current. In such a system, the member is directly responsive to current input. Other specific installations of this general type may be used. It will be understood that the invention is broadly applicable to thermostatic mechanisms where the manganese, nickel, copper alloys comprise the high expansion component of the differential expansion portion of such mechanisms which utilize a difference in the thermal expansion of two or more materials.

The composition of the alloys used in accordance with my present invention, where the various properties discussed may be obtained, is clear from the description alone as well as when taken with the drawings. The several properties obtainable should obviously be considered in the design of a control element. The drawings show that at least 10% manganese should be present, but that the manganese may comprise in some cases as much as 97% of the whole. The proportion of copper may be varied greatly as well, but the nickel content should not be more than 70% of the total composition. One satisfactory group of alloys comprises those containing from 3% to 26% nickel, from 2% to 25% copper, and from 67% to 80% manganese, the total of said metals amounting to substantially 100%. Another range of excellent properties comprises those alloys containing from 8% to 20% nickel, from 7% to 19% copper, balance substantially all manganese, especially electrolytic manganese of high purity. A particularly satisfactory group of alloys comprises those containing from about 70% to 75% manganese, from about 8% to about 15% nickel, and from about 15% to 20% copper. Of especial value is an alloy of about 72% manganese, about 10% nickel and about 18% copper, particularly when prepared from highly pure metals, preferably those produced electrolytically. Electrolytic manganese of at least 99.0% and preferably of the order of 99.9% purity is especially satisfactory in the preparation of the high expansion alloys used in accordance with the present invention.

This application is a continuation-in-part of my application Serial No. 303,006, filed November 6, 1939.

60 What I claim as new and desire to protect by Letters Patent of the United States is:

1. As a new article of manufacture, a control member adapted to expand and contract on heating and cooling, respectively, comprising metallic members having different expansion characteristics, one of said members being made of an alloy of manganese, nickel and copper, said alloy having a temperature coefficient of expansion greater than  $20 \times 10^{-6}$  cm./cm./degree C. and comprising from 67% to 80% manganese, from 3% to 26% nickel, and from 2% to 25% copper, the total of the manganese, copper and nickel amounting to substantially 100%.

2. As a new article of manufacture, a control member adapted to expand and contract on heat-

ing and cooling, respectively, comprising metallic members having different expansion characteristics, one of said members being made of an alloy of manganese, nickel and copper, said alloy having a temperature coefficient of expansion greater than  $20 \times 10^{-6}$  cm./cm./degree C. and comprising from 8% to 20% nickel, from 7% to 19% copper, and the balance of said alloy being substantially all manganese, the total of the manganese, copper and nickel amounting to substantially 100%.

3. As a new article of manufacture, a control member adapted to expand and contract on heating and cooling, respectively, comprising metallic members having different expansion characteristics, one of said members being made of an alloy of manganese, nickel and copper, said alloy having a temperature coefficient of expansion greater than  $20 \times 10^{-6}$  cm./cm./degree C. and comprising from 70% to 75% manganese, from 8% to 15% nickel, and from 15% to 20% copper, the total of the manganese, copper and nickel amounting to substantially 100%.

4. As a new article of manufacture, a control member adapted to expand and contract on heating and cooling, respectively, comprising metallic members having different expansion characteristics, one of said members being made of an alloy of nickel, copper and manganese, said alloy having a temperature coefficient of expansion greater than  $20 \times 10^{-6}$  cm./cm./degree C. and comprising about 10% nickel, about 18% copper, and about 72% manganese.

5. As a new article of manufacture, a control member adapted to expand and contract on heating and cooling, respectively, comprising metallic members having different expansion characteristics, one of said members being made of a high nickel-iron alloy having a low coefficient of linear expansion, and another of said members being made of an alloy of nickel, copper and manganese, said alloy having a temperature coefficient of expansion greater than  $20 \times 10^{-6}$  cm./cm./degree C. and comprising about 10% nickel, about 18% copper, and about 72% manganese.

6. As a new article of manufacture, a control member adapted to expand and contract on heating and cooling, respectively, comprising metallic members having different expansion characteristics, one of said members being made of Invar and another of said members being made of an alloy of nickel, copper and manganese, said alloy having a temperature coefficient of expansion greater than  $20 \times 10^{-6}$  cm./cm./degree C. and comprising about 10% nickel, about 18% copper, and about 72% manganese.

7. As a new article of manufacture, a control member adapted to expand and contract on heating and cooling, respectively, comprising metallic members having different expansion characteristics, one of said members being made of Invar and the other one being made of an alloy of nickel, copper and manganese, said alloy having a temperature coefficient of expansion greater than  $20 \times 10^{-6}$  cm./cm./degree C. and comprising from 3% to 26% nickel, from 2% to 25% copper, and from 67% to 80% electrolytic manganese of at least 99% purity, the total of the nickel, copper and electrolytic manganese of said alloy amounting to substantially 100%.

8. As a new article of manufacture, a control member adapted to expand and contract on heating and cooling, respectively, comprising metallic members having different expansion characteristics, one of said members being made of a

nickel-iron alloy having of the order of at least 33% nickel and having a low coefficient of linear expansion, and the other one being made of an alloy of nickel, copper and manganese, said alloy having a temperature coefficient of expansion greater than  $20 \times 10^{-6}$  cm./cm./degree C. and comprising from 3% to 26% nickel, from 2% to 25% copper, and from 67% to 80% electrolytic manganese having a purity of the order of 99.9%, the total of the nickel, copper and electrolytic manganese of said alloy amounting to substantially 100%.

9. A bi-metal strip comprising a first metallic member made of Invar and a second metallic member of a composition and expansion properties different from those of the first metallic member, said second member being made from an alloy of nickel, copper and manganese, said alloy having a temperature coefficient of expansion greater than  $25 \times 10^{-6}$  cm./cm./degree C. and comprising from 3% to 26% nickel, from 2% to 25% copper, and from 67% to 80% manganese, the total of the nickel, copper and manganese amounting to substantially 100%.

10. As a new article of manufacture, a control member adapted to expand and contract on heating and cooling, respectively, comprising metallic members having different expansion characteristics, one of said members being made of a low expansion material and the other of said members being made of a high expansion material in the form of an alloy of manganese, nickel and copper, said alloy having a temperature coefficient of expansion greater than  $20 \times 10^{-6}$  cm./cm./degree C. and an electrical resistance of at least  $170 \times 10^{-6}$  ohms/cm.<sup>3</sup>, and comprising from 67% to 80% manganese, from 3% to 26% nickel, and from 2% to 25% copper, the total of the manganese, nickel and copper in said alloy amounting to substantially 100%.

11. As a new article of manufacture, a control member adapted to expand and contract on heating and cooling, respectively, comprising metallic members having different expansion characteristics, one of said members being made of Invar and the other of said members being made of a high expansion material in the form of an alloy of manganese, nickel and copper, said alloy having a temperature coefficient of expansion not substantially less than  $25 \times 10^{-6}$  cm./cm./degree C. and an electrical resistance of at least  $170 \times 10^{-6}$  ohms/cm.<sup>3</sup>, and comprising from 70% to 75% manganese, from 8% to 15% nickel, and from 15% to 20% copper, the total of the manganese, copper and nickel in said alloy amounting to substantially 100%.

12. A bi-metal strip comprising a first metallic member having a low coefficient of linear expansion and a second metallic member having a high coefficient of linear expansion, said second member being made from an alloy of nickel, copper and manganese, said alloy having a temperature coefficient of expansion greater than  $20 \times 10^{-6}$  cm./cm./degree C. and comprising from 70% to 75% electrolytic manganese having a purity of at least 99.9%, from 8% to 15% nickel, and from 15% to 20% copper, the total of the manganese, copper and nickel in said alloy amounting to substantially 100%.

13. A bi-metal strip comprising a first metallic member having a low coefficient of linear expansion and comprising an iron alloy containing a high proportion of nickel, and a second metallic member having a high coefficient of expansion, said second member being made from an alloy

of nickel, copper and manganese, said alloy having a temperature coefficient of expansion of at least about  $25 \times 10^{-6}$  cm./cm./degree C., and comprising from 8% to 20% nickel, from 7% to 19% copper and the balance of said alloy being substantially all electrolytic manganese of high purity, the total of the nickel, copper and electrolytic manganese in said alloy amounting to substantially 100%.

14. A bi-metal strip comprising a first metallic member made of Invar, and a second metallic member made from an alloy of nickel, copper and manganese, said alloy having a temperature coefficient of expansion of at least about  $25 \times 10^{-6}$  cm./cm./degree C., and comprising from 8% to 20% nickel, from 7% to 19% copper and the balance of said alloy being substantially all electrolytic manganese of high purity, the total of the nickel, copper and electrolytic manganese in said alloy amounting to substantially 100%.

15. Thermostatic metal comprising a plurality of joined metallic laminations, one of said laminations having a relatively high coefficient of expansion and comprising an alloy of the following constituents by weight: manganese in excess of 50% and up to about 90%, nickel 4% to 20%, balance substantially all copper, the copper comprising at least 5%; the other lamination having a relatively low coefficient of expansion.

16. In a device responsive to temperature changes to perform work or mechanical movement, a plurality of metallic members, one of said members having a relatively high linear coefficient of thermal expansion and comprising an alloy of the following constituents by weight: manganese in excess of 50% and up to about 90%, nickel 4% to 20%, balance substantially all copper, the copper comprising at least 5%; the other member having a relatively low linear coefficient of thermal expansion and comprising essentially "Invar," an alloy of iron and nickel.

17. Thermostatic metal comprising a plurality of joined metallic laminations, one of said lami-

nations having a relatively high coefficient of thermal expansion and comprising an alloy of the following constituents by weight: manganese 60% to 85%, nickel 5% to 30%, balance substantially all copper, the copper comprising at least 7%, the other lamination having a relatively low coefficient of thermal expansion.

18. A thermostatic metal comprising a plurality of joined metallic laminations, one of said laminations having a relatively high coefficient of thermal expansion and comprising an alloy consisting by weight of about 72% manganese, 18% copper, and 10% nickel, the other lamination having a relatively low coefficient of thermal expansion.

19. A thermostatic metal comprising a plurality of joined metallic laminations, one of said laminations having a relatively high coefficient of thermal expansion and comprising an alloy consisting by weight of about 72% manganese, 18% copper, and 10% nickel, the other lamination consisting of "Invar."

20. In a device responsive to temperature changes to perform work or mechanical movement, a plurality of metallic members, one of said members having a relatively high linear coefficient of thermal expansion and comprising an alloy of the following constituents by weight: manganese 60% to 65%, nickel 5% to 30%, balance substantially all copper, the copper comprising at least 7%, the other member having a relatively low linear coefficient of thermal expansion.

21. In a device responsive to temperature changes to perform work or mechanical movement, a plurality of metallic members, one of said members having a relatively high linear coefficient of thermal expansion and comprising an alloy of the following constituents by weight: manganese about 72%, copper about 18%, and nickel about 10%, the other member having a relatively low linear coefficient of thermal expansion.

REGINALD S. DEAN.